

## UNITED STATES PATENT OFFICE

HANS OSBORG, OF FRANKFORT-ON-THE-MAIN, GERMANY

PROCESS OF TREATING MOLTEN FERROUS METALS AND ALLOYS WITH COMPOSITIONS  
CONTAINING "LITHIUM-ALKALI" ALLOYS AND PRODUCTS RESULTING FROM SUCH  
TREATMENTS

No Drawing. Application filed December 21, 1931, Serial No. 582,490, and in Canada June 26, 1931.

The present invention relates to a process of treating iron-bearing metals and alloys in their molten state with an alloy of lithium and a metal of the "alkali" group, including alkali, and/or alkaline earth groups and/or rare earth group and to the improved products resulting from such a process.

Heretofore, a great variety of scavengers and improvers of metals and alloys have been proposed. Of these scavengers and improvers, the more important were manganese, silicon, aluminum, magnesium, metallic lithium, metallic calcium, etc. From an industrial point of view manganese, silicon, aluminum, magnesium, have been the most important, but the art was attempting to obtain better and more satisfactory results than those obtained by the use of these substances. With this object in view, those skilled in the art were attempting to find improved scavengers. Metallic lithium and metallic calcium were proposed, but it was found that these metals had short-comings and disadvantages when used on an industrial scale.

The more serious disadvantages were that the molten metal and alloy undergoing treatment was not cleaned completely, did not possess the desired improved properties and usually was contaminated with impurities or contained blow holes. In other words, when lithium or in fact some other metal of the alkali group or alkaline earth group was added to a molten bath of metal these disadvantages were encountered which in many cases not only counter-balanced any advantages but actually over-balanced any advantages. For instance, in the treating of steel or steel alloys, the temperature of the molten bath was such as to cause a quick volatilization of lithium with the consequence that the treatment only partly occurred or that an excessive amount of lithium had to be used in order to obtain the desired results. From a practical point of view, it was found that the use of these metals was not wholly economical and satisfactory on an industrial scale. Various suggestions have been made for remedying the shortcomings and disadvantages noted hereinabove with respect to prior scavengers including metallic lithium and

metallic calcium and/or processes of using the same, but as far as is known, no scavenger and/or improver and/or process of using the same has been proposed which is wholly satisfactory and practical when used on an industrial scale.

It is an object of the present invention to provide a process of treating iron-bearing metals and alloys in their molten state so as to obtain the benefits resulting from lithium treatments without the disadvantage noted hereinabove.

It is a further object of the invention to provide a simple, economical and thoroughly satisfactory process of treating iron-bearing metals and alloys in their molten state with active lithium-bearing substances so as to improve the characteristics thereof.

It is another object of my invention to provide a process of treating molten metals and molten alloys with an active lithium alloy of a metal of the alkali group or alkaline earth group or rare earth group which is capable of being carried into commercial practice on an industrial scale in the ferrous and the non-ferrous industries, which is also capable of producing greater effects than provided by the same amount of lithium and the like.

Other objects and advantages of the invention will become apparent from the following description.

Broadly stated, my invention contemplates the treatment of molten iron-bearing metals and alloys with an active lithium alloy of a metal of the alkali group or alkaline earth group or rare earth group in which the lithium is so bonded that the loss thereof through volatilization and the like is materially reduced. At the same time, the lithium alloy can function actively to effect improvements in the properties and qualities of the metallic substance under treatment. I have found that in carrying my invention into practice, that lithium alloys containing members of the alkali or alkaline earth families such, for example, as calcium, barium, strontium, magnesium, lanthanum, cerium, sodium or potassium or relatively stable compositions of lithium and silicon or of mixtures of the foregoing substances can be utilized in the

treatment of metals and alloys in their molten state so as to effect improvements in the properties and qualities in the metals or alloys treated.

5 The following examples are given for illustrative purposes and for a better understanding of carrying my invention into practice.

*A. Cast iron general*

10 It is well known, that cast iron has to serve many purposes which have different requirements. In all cast irons, however, one of the most important improvements which 15 the art has been attempting to make is an increase in the tensile strength of the cast iron, combined with a good density, a good machinability, etc. From a practical and commercial point of view, it is essential that 20 the improved cast iron does not cost much more than ordinary cast iron. If the cost of the improved cast iron is too high then it is unavailable economically.

At the present time conventional improved 25 cast irons are made generally by the use of two distinct methods; (1) an alloying method and (2) a heat treatment method of the molten metal.

In the first method, alloying elements such 30 as nickel, chromium, etc., are added either singly or in combination in addition to silicon, etc. If nickel is added, for instance, oxides of nickel are formed to a considerable extent and the benefit of the alloying element 35 included is diminished thereby. Moreover, there seems to be some doubt as to the effect of nickel on the dispersion of graphite. In some cases, the dispersion effect can be observed whereas in other cases it cannot be 40 observed. In the same way, the addition of the other alloying metals have limitations. Since the alloying effect of these additions, such as nickel or chromium is diminished by the gases, oxygen, and other impurities present in the molten metal, it is possible to greatly 45 improve the effect of nickel and chromium by treating molten cast iron with the present improved lithium alloy.

The second method of producing improved 50 cast iron contemplates overheating the cast iron while in a molten condition. This overheating effects a better dispersion of the graphite but has a detrimental effect of increasing the oxygen contained in the molten 55 metal. As is well known, when oxygen is present in cast iron, the density is considerably decreased. In other words, the cast iron is somewhat porous and cannot be dependent 60 upon for structural engineering purposes. For example, a cast iron containing 0.06 to 0.08% of oxygen has a slightly higher tensile strength than a cast iron without oxygen, but the density of the improved cast iron is 65 decreased about 0.02 to about 0.03 points or

units. This decrease in density is detrimental to the cast iron and limits the uses thereof.

When cast iron is treated according to the process of the present invention, it has been found that the cast iron has a very fine and even distribution of the graphite; that some of the free carbon has combined with the metal without making the cast iron too hard for machining purposes; that the gases and oxygen have been practically removed; that the crystal structure of the cast iron has been decidedly improved as shown by photomicrographs; that a general improvement of the mechanical properties have been effected (see following tables). Among the improvements 70 in cast iron treated with the present improved lithium alloy the following may be noted; the cast iron is sound, has a higher tensile strength than untreated metal from the same heat and has a very good machinability. The 75 test pieces of cast iron produced by the present invention, for example, turned on the lathe to give better and larger chips in spite of the fact that cast iron produced by the present invention has a higher hardness than ordinary cast iron. Moreover, the untreated cast iron was found to have "hard spots". By the use of the present process and the 80 present improved lithium alloy, the "hard spots" are eliminated and uniform cast iron 85 with uniform hardness is produced.

A comparison of the fractures of cast iron bars treated with the present improved lithium alloy and those untreated shows that cast iron produced by the present invention has a 90 finer grain structure than the other one and is of a lighter color which means that the graphite is broken up in finer particles and distributed more uniformly and, furthermore, that to some extent there is less graphitic carbon present.

The casting properties of the molten metal were improved. After the present improved lithium alloy was added to molten cast iron in a bull ladle, the temperature increased and 100 the fluidity was much better than that of untreated cast iron.

*B. Cast iron made in a cupola*

Photomicrographs of specimen clearly 115 show the improvement in cast iron when treated with the present lithium alloy. For purposes of comparison, photomicrographs of a corresponding cast iron which has been untreated were taken. For instance, photomicrographs (#223) were taken from a bar of ordinary gray cast iron which did not have any steel scrap added thereto and which was made in a cupola. The unetched and etched 120 photomicrographs show large flakes of graphite at the grain boundaries. It is well known that when the graphite occurs in large flakes at the boundary a weak cast iron results.

Some ordinary cast iron of the same heat 125

which had been treated with the present lithium alloy was made up in the form of test bars to form for example, a specimen (#226). The photomicrographs of this specimen show the improvement in the metal. The graphite flakes are broken up and finely distributed throughout the mass of cast iron. A comparison of the photomicrographs makes it self evident that beneficial improvements are effected by the use of the present lithium alloy.

Tests were made on ordinary gray cast iron and the same cast iron treated with the present lithium alloy and the following Table I gives the results of these tests. It should be noted that no addition was made to the cast iron, not even of the usual steel scrap.

Table I

| Property         | Untreated or treated in the usual way | Treated with the present lithium alloy |
|------------------|---------------------------------------|----------------------------------------|
| Tensile strength | 16000 #/sq. in.                       | 20000 #/sq. in.                        |
| Brinell hardness | 127                                   | 147                                    |
| Machinability    | Poor                                  | Very good                              |
| Crystals         | Large                                 | Very small                             |

The foregoing tests as well as the following tests on cast iron were made on a tensile bar and not on a so-called arbitration bar. It is to be noted that if an arbitration bar, which is the usual commercial practice, were used, higher figures for tensile strength would, of course, have been obtained.

A cast iron containing nickel and steel scrap is usually recommended as a good product. If, however, nickel cast iron is treated with the present lithium alloy, then more accentuated improvements are obtained as shown by photomicrographs taken of test specimens and data obtained in testing specimens. For instance, ordinary untreated cast iron containing 40% steel scrap and 1% nickel showed a tensile strength of 26,000 #/sq. in. The photomicrograph disclosed large graphite flakes and large white areas of ferrite and phosphide eutectic. On the other hand, the same cast iron from the same cupola when treated with the present lithium alloy showed a tensile strength of about 30,000 #/sq. in. and the photomicrograph disclosed a fine distribution of graphite and white areas.

#### C. Cast iron made in an electric arc furnace

Cast iron was made in an electric arc furnace with plain gray iron scrap with no addition even of steel scrap by heating the furnace up to 2800° F. and holding it at this temperature for about fifteen minutes. From this heat cast iron specimens were made which were untreated and cast iron specimens were made which were treated with the present lithium alloy.

The aforesaid specimens were subjected to

tests and Table II shows the results of these tests:

Table II

| Specimen No. | Tensile strength    | Brinell hardness | Treatment                      | 70 |
|--------------|---------------------|------------------|--------------------------------|----|
| 232-----     | #/sq. in.<br>27,000 | Number<br>187.5  | Untreated.                     | 75 |
| 233-----     | 32,000              | 207.5            | Treated with present Li Alloy. |    |
| 234-----     | 30,000              | 207.5            | Do.                            |    |

Photomicrographs showed that an untreated specimen (#232) had many hard spots and showed non-uniformity of material whereas photomicrographs showed that treated specimens (#233 and #234) possessed a uniform structure, and that there was an excellent distribution of the graphite in the form of very fine particles. Tests demonstrated that the treated specimens exhibited excellent machinability.

Ordinary untreated gray cast iron of a high grade containing no addition of steel scrap, etc. produced by the overheating method shows tensile strength of about 23,000 to about 25,000 #/sq. in. The ordinary cast iron mentioned above had a tensile strength still higher than the best of the usual commercial gray cast iron. The foregoing table demonstrates that cast iron, when treated with the present lithium alloy, gives far greater tensile strength than the best of the untreated ordinary cast iron. Thus improvements of the order of about 12 to 18% over the best ordinary cast iron without even using nickel or chromium or steel scrap have been obtained by the use of the present invention.

#### D. Carbon steel

Carbon steel was made in accordance with the usual and conventional practices and specimens of the thus-produced ordinary carbon steel were obtained. A portion of the heat of the aforesaid carbon steel was treated in accordance with the principles of the present invention and specimens were made from the thus-treated carbon steel. The following Table III shows the results of some tests of these specimens:

Table III

| Carbon                 | Tensile strength         | Brinell hardness    | Remarks                                                                                                                                                        | 120 |
|------------------------|--------------------------|---------------------|----------------------------------------------------------------------------------------------------------------------------------------------------------------|-----|
| (A) .3-----            | #/sq. in.<br>50,000----- | Number<br>98.5----- | Untreated (somewhat dirty).                                                                                                                                    | 125 |
| (B) .3-----            | 65-70,000-----           | 119-----            | Treated (clean) from same heat as (A) 40-45,000 #/sq. in. yield point, 30-33,000,000 modulus of elasticity. About 35% elongation. About 45% reduction of area. |     |
| (C) .5-----<br>.6----- | 105,000-----             | 207.5-----          | Untreated (good quality) elastic limit 30,000 lbs./sq. in. Elongation 3%. Reduction of area 2.7%.                                                              |     |
| (D) .5-----<br>.6----- | 108,000-----             | 207.5-----          | Treated (good quality) elastic limit 53,000 lbs./sq. in. Elongation 7%. Reduction of area 11.5%.                                                               | 130 |

## (A) to (D) tested in the annealed condition

Photomicrographs of the aforesaid specimens demonstrated that the improved carbon steel embodying the present invention had a better structure, fewer inclusions, a more uniform pearlitic constitution, etc., than ordinary untreated carbon steel.

## E. Alloy steels

10 Various types of nickel-chromium and chromium steels were treated with the present lithium alloy. In general, the treatment resulted in the increase of temperature of the molten metal; better fluidity of the molten bath of metal; better castings; improved crystal structure; cleaner metal; superior metal regarding physical and mechanical properties and an increase in corrosion resistance. All tests were carried out on a comparative basis between untreated metal and the same metal when treated in accordance with the present invention.

Photomicrographs of improved alloy 25 steels embodying the present invention will clearly show to one skilled in the art the improvements obtained by the use of the present lithium alloy. These improvements include better structure, fewer and smaller inclusions, 30 practically complete freedom from impurities at grain boundaries, etc.

Various nickel-chromium steels which had been treated in accordance with the present invention were subjected to tests. The following Tables IV, V and VI show the results of these tests:

Table IV

Tests on a steel containing 18% Cr and 8% Ni and treated with 0.02% Lithium-Alkali Alloy (Li-Ca)

| 40 | Size           | Elastic limit<br>#/sq. in. | Tensile strength<br>#/sq. in. | Per cent elongation in 2" | Per cent reduction in area | Modulus of resilience | Brinell Hardness number |
|----|----------------|----------------------------|-------------------------------|---------------------------|----------------------------|-----------------------|-------------------------|
|    |                |                            |                               |                           |                            |                       |                         |
| 45 | 2" Sq.*        | 39400                      | 80200                         | 15.0                      |                            | 25.6                  | 165.5                   |
|    | 1" Sq.*        | 44000                      | 112000                        | 34.0                      |                            | 28.1                  | 176.0                   |
|    | 1/4" Rd.       | 54000                      | 135000                        | 15.0                      |                            | 51.3                  | 238.0                   |
|    | 5/8" Rd.       | 82000                      | 160000                        | 11.5                      |                            | 129.1                 | 314.0                   |
|    | .125" 1/8" Rd. | 102500                     | 240000                        | 4.5                       |                            | 235.7                 |                         |
|    | .07" Rd.       | 130000                     | 263750                        |                           | 34.8                       | 369.5                 |                         |
| 50 | .06" Rd.       | 162500                     | 303500                        |                           | 24.8                       | 517.5                 |                         |

Table V

Tests on a steel containing 18% Cr and 8% Ni and Treated with 0.04% present lithium Alkali-Alloy (Li-Ca)

| 55 | Size           | Elastic limit<br>#/sq. in. | Tensile strength<br>#/sq. in. | Per cent elongation in 2" | Per cent reduction in area | Modulus of resilience | Brinell Hardness number |
|----|----------------|----------------------------|-------------------------------|---------------------------|----------------------------|-----------------------|-------------------------|
|    |                |                            |                               |                           |                            |                       |                         |
| 60 | 2" Sq.*        | 38000                      | 77200                         | 18.0                      |                            | 19.2                  | 143.5                   |
|    | 1" Sq.*        | 44000                      | 113400                        | 36.0                      |                            | 31.9                  | 176.0                   |
|    | 1/4" Rd.       | 57000                      | 134300                        | 18.0                      |                            | 57.0                  | 267.0                   |
|    | 5/8" Rd.       | 95000                      | 167800                        | 12.0                      |                            | 209.5                 | 341.0                   |
|    | .125" 1/8" Rd. | 110000                     | 251600                        | 4.0                       |                            | 255.9                 |                         |
|    | .07" Rd.       | 109300                     | 267700                        |                           | 30.6                       | 254.0                 |                         |
| 65 | .06" Rd.       | 123400                     | 288650                        |                           | 24.7                       | 320.0                 |                         |

\*NOTE.—The values for the two larger sizes would be in fact still higher because due to a mistake in the mill the ingots were not cropped at all. Therefore, these sizes had a defect known as pipes.

Table VI

Nickel chromium steels, comparative figures as obtainable from the industries

(A) Radiator shells, as used for Ford automobiles, (18% Cr 8% Ni steel)

|                       | #/sq. in. |
|-----------------------|-----------|
| Tensile strength..... | 90,000    |
| Elastic limit.....    | 42,000    |

(B) Alleghany wire (average quality of 18% Cr 8% Ni steel)

|                 | #/sq. in.                |
|-----------------|--------------------------|
| .035" Diam..... | 92,000 tensile strength  |
| 0.01" Diam..... | 48,000 elastic limit     |
| 0.01" Diam..... | 117,000 tensile strength |
| 0.01" Diam..... | 60,000 elastic limit     |
| 0.01" Diam..... | 143,000 tensile strength |
| 0.01" Diam..... | 75,000 elastic limit     |

Alleghany strip (Cold rolled from .078 gauge down to .049 gauge)

|  | #/sq. in. tensile strength    |
|--|-------------------------------|
|  | 157,850 #/sq. in. yield point |
|  | 153,460 #/sq. in. yield point |

(C) Krupp-Nirosta KA2 hot rolled sheet steel

|  | #/sq. in.                |
|--|--------------------------|
|  | 111,000 tensile strength |
|  | 56,000 elastic limit     |

(D) Bethlehem steel (18% Cr and 8% Ni when cold drawn from 1/4" to 1/8")

|  | #/sq. in. tensile strength    |
|--|-------------------------------|
|  | 174,000 #/sq. in. yield point |
|  | 167,000 #/sq. in. yield point |
|  | 302 BHN hardness.             |

The following Table VII shows the results of tests applied to a nickel-chromium steel in the cast condition. Specimens of untreated nickel-chromium steel were made and corresponding specimens of material were taken from the same heat after treatment with the present alloy. The tests showed the following results:

Table VII

(18% Cr 8% Ni steel) as cast

| Property                         | Untreated       | Treated         |
|----------------------------------|-----------------|-----------------|
| Tensile strength per sq. in..... | 61900 #/sq. in. | 72350 #/sq. in. |
| Elongation in 2".....            | 18%             | 29%             |
| Brinell hardness number.....     | 134.5           | 181.5           |

## Example No. 1

In the treatment of iron or steel, for instance the molten metal is contained in a suitable crucible such as a graphite crucible or in a bull ladle or in an ingot mold. To the molten mass I add in any appropriate manner, an active lithium alloy, for example, an alloy of lithium and calcium in an amount sufficient to effect improvements in the properties of the iron or steel. In practice, I have found that up to about 2 parts of an alloy of lithium and calcium having about 50% lithium content are capable of effectively treating about 100 parts of molten steel or steel alloys.

The addition of the active lithium alloy to the molten metal is preferably effected by plunging the selected amount of active lithium

um alloy into the molten material in a crucible by any appropriate means such as an inverted cup with side openings or ports or the like. By adding the active lithium alloy to the 5 molten metal in the aforesaid manner, I am able to effect a thorough distribution of the lithium alloy throughout the molten mass and to effect the proper treatment of said metal to improve the properties and qualities there-  
10 of.

When iron and/or steel and/or alloys thereof are treated with one of my active lithium-bearing alloys, the molten mass has a better fluidity and consequently, can be cast 15 very much better than heretofore and gives better and denser castings. In addition, the physical properties of the iron or steel or metal or alloy treated are improved. For instance, there is an increased hardness and 20 corrosive resistance of the metal thus treated and the finished product is relatively or practically free from blow holes, oxygen, sulphur and the like.

25 *Example No. 2*

When steel or a steel alloy is used for the production of castings, I add to about 100 parts of molten iron prior to casting enough 30 of a lithium alloy such as a lithium-calcium alloy or a mixture of lithium alloys having such a composition as to give a lithium content up to about 1%. The lithium alloy is preferably added in the form of a solid briquette, block, lump or the like which is introduced into the body and preferably the 35 lower portion of the molten mass of iron by means of an inverted cup or other appropriate instrumentality. The lithium alloy thus added, improves the crystal structure of the 40 steel; combines with gases, such as oxygen and nitrogen, and also with such detrimental substances as sulphur and phosphorus; increases the fluidity of the molten steel and produces denser and sounder castings than 45 produced heretofore. In practice, I prefer in some instances to add the lithium alloy in a mass which is surrounded by or coated with iron silicide. By adding the lithium 50 alloy in this manner, the procedure is facilitated. If it is desired, a lithium-calcium alloy can be silicided and then the silicided lithium alloy used for the treatment of the 55 molten metal or alloy.

Instead of steel or iron in the examples 55 given above, nickel or alloys thereof or copper or alloys thereof can be treated by the addition of the lithium alloy to the molten metallic mass. Sufficient lithium-bearing 60 substance is added to the molten mass to give the latter a lithium content up to about 1.0%.

In some instances, I prefer to employ an 65 alloy of lithium with the metal or alloy to be treated. For example, if steel is to be treated, I use an active lithium alloy containing iron. The lithium alloys should prefer-

ably be silicided or reacted with silicon prior to use.

The amount of lithium alloy added to the molten metallic mass depends upon a number of variables as one skilled in the art will readily understand. For example, the percentage of lithium in the lithium alloy will determine in part how much of the substance is to be used. Then again the amount of impurities and gases in the molten metal or 70 alloy and the improvement to be given to the metal or alloy will also have to be taken into account in determining the amount of lithium-bearing substance to be used.

It will be observed that the present invention provides a process which can be utilized on an industrial scale to produce successful and satisfactory results which are acceptable to those skilled in the art.

It will be further observed that the present invention provides a method for the production of improved metals and alloys which not only can be carried out on a laboratory scale but which also can be carried out on an industrial scale. When carrying the invention out on an industrial scale the preferred addition of the lithium alloy is an amount within the range of about 0.005% to about 0.05%.

It will also be noted that the present invention provides a process by the use of which the disadvantages inherent in the sole use of lithium alone or other member of the alkali group or the alkaline earth group alone are avoided and unexpected advantages are obtained from the use of lithium alloys of 90 metals of the alkali group or the alkaline earth group. The lithium in alkali alloys contemplated by my invention is exceedingly active and have an activity which could not be predicted from the prior use of 95 lithium alone of other metals of the alkali or alkaline earth groups alone.

Although I have herein described specific 100 illustrative examples of my invention which included specific substances, percentages and the like, it is to be observed that the invention is not to be limited thereto but the scope and spirit thereof is to be determined by the appended claims. For instance, when in the 105 specification and claims, I use the term "lithium-alkali alloy" it is intended to mean lithium alloy of a metal of the alkali group or alkaline earth group or rare earth group. Similarly, when the term "alkali" is used, it is 110 intended to refer to alkali group, alkaline earth group or rare earth group.

The present application is a continuation 115 in part of my co-pending application, Serial No. 467,625, filed July 12, 1930, entitled "Processes of treating molten metals and alloys 120 with compositions containing lithium and products resulting from such treatment."

What is claimed is:

1. The process of treating iron and/or steel 125 and/or alloys thereof in their molten state

- to improve the properties thereof, which comprises treating said iron and/or steel and/or alloys thereof while in a molten state with a "lithium-alkali" alloy.
- 5 2. The process set forth in claim 1 in which the "lithium-alkali" alloy contains lithium and calcium.
3. The process set forth in claim 1 in which up to about 2 parts of the "lithium-alkali" 10 alloy is used to about 100 parts of iron and/or steel and/or alloys thereof.
4. The process of treating iron and/or steel and/or alloys thereof in their molten state to improve the properties thereof which comprises dipping a solid body of an active "lithium-alkali" alloy into a molten mass of iron and/or steel and/or alloys thereof to be treated and stirring the thus treated molten mass to effect a thorough distribution of said 15 20 "lithium-alkali" alloy.
5. The process of treating iron and/or steel and/or alloys thereof in their molten state to improve the properties thereof which comprises adding a briquette containing an active 25 "lithium-alkali" alloy to the lower portion of a molten mass of iron and/or steel and/or alloys thereof to be treated and causing a thorough mixing of said lithium alloy in said molten iron and/or steel and/or alloys 30 thereof.
6. The process of treating iron and/or steel and/or alloys thereof in their molten state to improve the properties thereof which comprises adding a lithium-calcium alloy to 35 a molten mass of iron and/or steel and/or alloys thereof to be treated and stirring said molten mass to effect a treatment of the various parts of said mass with said lithium-calcium alloy.
- 40 7. The process of treating iron and/or steel and/or alloys thereof in their molten state to improve the properties thereof which comprises dipping a block of lithium-calcium alloy into the lower portion of a molten 45 mass of the iron and/or steel and/or alloys to be treated and effecting a distribution of said lithium-calcium alloy substantially throughout said mass.
8. The process of treating iron and/or 50 steel and/or alloys thereof in their molten state to improve the properties thereof which comprises adding a lithium alloy containing an "alkali" metal to a molten mass of metal or alloy to be treated and stirring said molten 55 mass to effect a treatment of the various parts of said mass with said lithium alloy containing an "alkali" metal.
9. The process set forth in claim 8 in which the lithium alloy is coated with lithium.
- 60 10. The improved iron and/or steel and/or alloy thereof which comprises an iron and/or steel and/or alloy thereof resulting from the treatment thereof in a molten state with a "lithium-alkali" alloy.
- 65 11. The improved iron and/or steel and/or alloy thereof as set forth in claim 10 in which the active lithium alloy is a lithium calcium alloy.
12. An article of manufacture comprising an improved iron and/or steel and/or alloy 70 thereof containing residual "lithium-alkali" alloy.
13. An article of manufacture set forth in claim 12 in which the "lithium-alkali" alloy comprises lithium and calcium.
- 75 In testimony whereof I have hereunto set my hand.
- HANS OSBORG.
- 80
- 85
- 90
- 95
- 100
- 105
- 110
- 115
- 120
- 125
- 130